

## UNITED STATES PATENT OFFICE.

RALPH R. PARISH, OF WATERBURY, CONNECTICUT, ASSIGNOR TO CHASE ROLLING MILL CO., OF WATERBURY, CONNECTICUT, A CORPORATION.

## METHOD OF PICKLING BRASS.

1,106,107.

Specification of Letters Patent.

Patented Aug. 4, 1914.

No Drawing.

Application filed January 12, 1914. Serial No. 811,741.

*To all whom it may concern:*

Be it known that I, RALPH R. PARISH, a citizen of the United States, residing at Waterbury, in the county of New Haven and State of Connecticut, have invented a new and useful Improvement in Methods of Pickling Brass; and I do hereby declare the following to be a full, clear, and exact description of the same.

- 10 As the art of making rolled or wrought brass has heretofore been practised, a certain percentage of inferior stock has been produced, owing to the imperfect pickling of the brass after annealing it, due to the fact 15 that the pickling solutions heretofore employed have been so far ineffective in their operation that they have left upon the surfaces of the pickled brass some irregular film-like deposits or blotches of pure or 20 relatively pure copper which appear in the finished product in the form of so called "stains," which, as the process proceeds, step by step, are rolled into the metal and produce unsightly and unworkable areas. 25 All such "stained" sheet brass is classed as inferior stock.

The object of my invention is to avoid these objections by improving brass pickling solutions so that they will be more effective and prevent the appearance upon the brass of any disfiguring films or deposits of pure or relatively pure copper.

With these ends in view, my invention consists in a brass pickling solution reinforced by a per acid or a derivative thereof, which dissolves the copper and copper oxids of whatever nature, formed upon the surfaces of the metal during the process of annealing.

40 My invention further consists in a brass pickling solution and a certain method as will be hereinafter described and pointed out in the claims.

It is well understood in brass mills, that 45 owing to a great variety of causes, superficial deposits of copper or copper oxids or both appear upon the brass during the successive annealing operations. Under perfect conditions of annealing, these objectionable deposits upon the brass do not occur, but they are so liable to occur, and so excessively difficult to control, that it is necessary to provide for removing them when they do occur in order to secure a product entirely of the

first grade of rolled brass. Provision is therefore always made in brass mills for pickling the brass immediately after it has been annealed. The pickling solution generally employed consists of a solution of about 10% of sulfuric acid in water. My

invention consists in introducing into such a pickling solution, a sufficient amount of a per acid, or a derivative of a per acid, to aid the sulfuric acid in the solution in attacking and dissolving the objectionable surface disfigurements, whatever the character of the same may be. On this point it may be said that a great many factors not necessary to here rehearse vary the amount and character of the disfigurements or blotches, such,

for instance, as the composition of the brass itself, the character, condition and mode of operating the annealing furnace used, the character of the fuel employed, the draft of the furnace and so on. In practising my invention, I may employ any suitable per acid or any suitable per acid derivative, such as per-sulfuric acid  $H_2S_2O_8$ , per-selenic acid  $H_2Se_2O_8$ , per-chromic acid  $CrO_3H_2O_2$  or any of the salts derived from such acids. The

amount of the per acid or per acid derivative used will be gaged according to the speed at which it is intended the pickling operation shall proceed. I have obtained good results by an amount of per acid or per acid derivative equivalent to about ten per cent. of the sulfuric acid content of the pickling solution.

The per-acids above referred to are what are chemically known as true per-acids defined by so eminent an authority as T. Slater Price in his monograph on "Per-Acids and Their Salts," (London 1912) "as those which are either formed by the action of hydrogen peroxid on ordinary acids, or else give rise to hydrogen peroxid on treatment with dilute sulfuric acid." To this generalization Price makes but one exception in this language: "In the case of persulfuric acid,  $H_2S_2O_8$ , chlorsulfonic acid has to be used, and not sulfuric acid." I would have it understood that in employing the term "per-acid" in the text and claims of my application, I use it in the sense in which the term is defined as above by Price.

I claim:—

1. A pickling solution for removing disfiguring blotches appearing upon annealed

41 brass, the said solution consisting of a sulfuric acid solution reinforced by a per-acid or a derivative thereof.

5 2. A pickling solution for removing dis-  
figuring blotches appearing upon annealed brass, the said solution consisting of a sulfuric acid solution reinforced by a per-sul-  
furic acid or a derivative thereof.

41 3. A method of pickling annealed brass  
10 consisting in subjecting it to the action of

a pickling solution of sulfuric acid which has been reinforced by a per-acid or a derivative thereof.

In testimony whereof, have signed this specification in the presence of two subscr- 15  
ing witnesses.

RALPH R. PARISH.

Witnesses:

FREDERIC C. EARLE,  
CLARA L. WEED.

Copies of this patent may be obtained for five cents each, by addressing the "Commissioner of Patents,  
Washington, D. C."